

H. E. TAYLOR.

## METHOD OF AND APPARATUS FOR SEGREGATING MINERALS.

APPLICATION FILED APR. 7, 1913.

1,248,948.

Patented Dec. 4, 1917.



Witnesses:  
P. M. Pezzetti  
J. S. Clarke.

Inventor:

Hiram E. Taylor

by Wright Brown Remond May  
201

## Attys.

# UNITED STATES PATENT OFFICE.

HIRAM E. TAYLOR, OF NORTH ADAMS, MASSACHUSETTS, ASSIGNOR TO NATIONAL METALS COMPANY, OF PHOENIX, ARIZONA, A CORPORATION OF ARIZONA.

## METHOD OF AND APPARATUS FOR SEGREGATING MINERALS.

1,248,948.

Specification of Letters Patent.

Patented Dec. 4, 1917.

Application filed April 7, 1913. Serial No. 759,411.

To all whom it may concern:

Be it known that I, HIRAM E. TAYLOR, a citizen of the United States, and resident of North Adams, in the county of Berkshire 5 and State of Massachusetts, have invented certain new and useful Improvements in Methods of and Apparatus for Segregating Minerals, of which the following is a specification.

10 This invention has for its object to furnish an efficient and economical method of separating metals or other elements or compounds from the ores in which such substances are found in nature, and also to provide an apparatus capable of carrying the invention into effect. The manner in which I accomplish this object is described in detail in the following specification and particularly pointed out in the appended claims.

15 The present invention includes steps of the operation and features of the apparatus described and illustrated in my prior application, Serial No. 608,173, filed February 11, 1911, with certain additional steps and features, and in so far as the disclosure herein corresponds to my prior application referred to, this application is a continuation of the prior one.

20 In the accompanying drawings, Figure 1 represents in elevation, a form of apparatus suitable for carrying my method into effect, and including the features in which one portion of my invention resides.

25 Fig. 2 is a detail view showing a possible form of one of the elements of the apparatus.

The same reference characters indicate the same parts in all the figures.

30 I will first describe the particular apparatus herein illustrated and then explain the principles according to which it operates and the method carried out thereby. In the drawing 1 represents a table or support on which is mounted a volatilizing furnace 2, or a plurality of such furnaces. In the 35 drawing, one furnace only is shown for illustration and this one is to be considered as typical of all where more than one are used. The furnace is electrical in character and the heat is furnished by an electric arc produced 40 between carbon pencils. There may be one or more pairs of complementary pencils, the drawing herein showing three pairs. They are indicated by the characters 3 and 4, the positive electrodes or carbon pencils being 45 designated 3 and the negative ones 4. They

50 pass through the inclosing walls of the furnace 2, which walls are made of or lined with, refractory material such as tile or fire brick, etc. The pencils are adjustably mounted in holders 5, 6 respectively whereby they may be adjusted to produce the proper sort of arc. They are arranged in vertical series where more than one pair are used, whereby a vertical zone of intense heat 55 of as great a length as required may be maintained.

From the furnace a conduit 7 rises and connects with a transfer pipe 8 which opens into a condensing chamber 9, into which a spray of water is projected by a sprinkler 70 10 fed by a pipe 11. A pipe 12 leads from the bottom of the condensing chamber and is led to a tank 13, supported at a level higher than the condensing chamber, from which the pipe 11 extends and is fed by 75 gravity. A pump 14 takes the liquor issuing from the bottom of the condensing chamber and delivers it into the tank 13. It will be noted that the transfer pipe 8 is very short and runs directly from the furnace to the 80 condensing chamber, which latter is very near to the furnace. This propinquity of the furnace and condensing chamber and the brief extent of the transfer pipe enable the 85 volatile products of the furnace to be delivered into the condensing chamber before they have had time to become cooled or condensed to any appreciable extent.

The ore to be treated is placed in a funnel, hopper, or other suitable container 15, from 90 which a pipe 16 leads downwardly into the furnace and terminates directly above the arc so as to discharge its contents into the zone of most intense heat.

95 The method or process in which my invention resides, in the carrying out of which I use the apparatus above described, may now be understood. Broadly stated it consists, first and essentially in bringing the volatile products of a part, or all, of the ore, or of the ingredients of the ore, obtained by heating, into such intimate mingled or mixed relation with a suitable liquid, that such volatile products are apparently absorbed by the liquid, and a resultant liquor is produced, which exhibits many of the characteristics of a solution. This is accomplished, with the apparatus here illustrated, by feeding metal bearing, or other, ore to the arc produced between 100 105 110

the carbon pencils 3, 4, volatilizing said ore by the heat of the arc, conducting the products of volatilization into the condensing chamber 9, mixing the products of volatilization while in substantially the condition in which they are produced with a certain liquid solvent, which I will presently name, and delivering the liquor consisting of this solvent with such products contained 5 therein, through the pipe 12 under propulsion of the pump 14 to the tank 13. This liquor may be further enriched with the constituents of the ore by being circulated again and again through the condensing 10 chamber and pump, thereby receiving constant additions to the vaporous matter already absorbed.

Although the only means I have thus far described for volatilizing is the electric arc, 20 yet I desire to make clear that my invention is not limited to volatilizing the ore by the electric arc or in an electric furnace. On the contrary, so far as the conversion of the raw material into the gaseous or vaporous state, 25 is concerned, the use of any other means capable of accomplishing the same or equivalent results, however employed, is within the scope of my invention and is intended to be covered in the following claims. That is, 30 since the main object of my invention is to produce a liquor containing volatile products liberated or produced from ore through the action of heat, it is not material to that aspect of the invention by which particular 35 heating means such volatile products are produced, nor whether such volatile products are of the same chemical composition as the natural ore or are of different composition, nor whether or not all of the constituents or ingredients of the ore are converted 40 into a volatile condition. I consider that the method of absorbing in a solvent the volatile constituents or products delivered or produced from ore, in substantially the condition 45 in which they are thus produced, whether produced by the ordinary processes of smelting, or by the heat of an electric arc, or in any other way, is within the scope of my invention and is covered by the appended 50 claims.

The solvent which I use is acidulated water, having as its acid principle, various acids suited to the character of ore treated. In treating ores of base metals such as copper, tin, zinc, lead, and the like, I may use hydrochloric acid, while for treating ores containing precious metals I may use aqua regia. In practice I have found it suitable in making the hydrochloric acid solution, to 55 use the concentrated acid of commerce in the proportions of about one ounce (or more) to twenty quarts of water. In practice also I have used aqua regia composed of three parts of hydrochloric acid to one part of 60 nitric acid, these being the concentrated

acids of commerce. The aqua regia so made, I have mixed with water in the same strength, that is, one ounce (or more) to twenty quarts of water. These proportions of water and acid are not fixed and invariable, but, on the contrary, a latitude in the strength of the solvent may be permitted according to the character of the ore treated, it being desirable that the solvent be of sufficient strength to dissolve at least a part of 70 the metal constituent of the ore, in the volatile state, and any acid solution having such strength is within the scope of this invention. I have found in practice that comparatively weak acid solutions will readily 75 absorb the products into which the ore is converted by this treatment.

Preferably acid-proof material is employed as far as possible in the construction 80 of the apparatus.

The ore, preferably pulverized to a fineness sufficient to pass through a screen having forty or more meshes to the inch, and being thereby brought to a sufficiently fine granular condition, upon being fed into the 90 furnace, is instantly volatilized when it enters the intense heat of the electric arc. The size of the carbon pencils and the number of superposed pencils are governed by the character of the ore treated and the rate at which 95 the ore is supplied, and are designed to produce a zone of heat of sufficient intensity and extent to volatilize as much of the ore as possible, and as rapidly as possible.

The vacuum maintained in the condensing 100 chamber by the sudden cooling and condensation of the products of volatilization and the pumping out of the liquor, induces flow of practically all of said products through the conduits 7 and 8. Said products enter the condensing chamber at a point below the top thereof, and the sprinkler 10 is above this point. Hence the solution introduced as a spray falls into the products from the furnace, and carries them down to 110 the bottom of the chamber. The location of the sprinkler, above the point at which the products from the furnace enter the condensing chamber, is an important feature, as it secures a more efficient mingling of the 115 volatile matter with the spray, and insures that all of the volatile products which enter the condensing chamber are washed to the bottom of the chamber.

A convenient form of sprinkler for these 120 purposes is shown at Fig. 2 and consists of a cup having a concave bowl 28 suspended across the open end of the pipe 11. The suspension means includes a strap 29, clamped to the pipe and has separated arms 125 30 connecting the strap with the cup. This sprinkler or sprayer may be adjusted to the most convenient point on the pipe.

Another feature of importance is that the pump 14 also serves the function of an agi- 130

tator which stirs the liquor and intimately mixes and mingles the liquid and volatile products together. I have found in practical experience that a mechanical agitation 5 of the liquid and volatile products together is, if not essential, at least very efficient in effecting an absorption of the volatile products by the liquid, and that, although without agitation it is in many cases difficult to 10 cause the liquor to retain the volatile products, yet with agitation the absorption of such products by the liquor is accomplished without difficulty. When the volatile products have been thus absorbed they are 15 retained in the liquor with a tenacity resembling that with which soluble substances are retained in solution by their solvents. While the pump as above described thus constitutes a means for agitating 20 and mixing the volatile matter and liquor, it is not the only means which could be used for this purpose, and therefore I include within my invention the step of causing an absorption of the volatile matter 25 by the liquor through agitation produced in any manner and by any means whatever suited to the purpose. I also prefer to make the pump 14 of such construction or character that it is capable of pumping 30 gases, as well as liquids. Such a pump is effective for performing the functions of both an agitator and a pump.

I have found, in practice, that when liquor produced in the manner described, by 35 action upon some sorts of ore has been allowed to stand for a considerable length of time, a sediment has settled on the bottom of the container, leaving the liquor transparent, while in other cases the liquor has 40 been clear from the beginning, with apparently no sediment. When such liquor is treated by the addition of alkali a precipitate is instantly formed.

A secondary part of my invention 45 consists in the step of recovering the desired elements or ingredients of the ore from the liquor in which they have been entrapped by the methods hereinbefore described. Many modes of treating the liquor to accomplish this end may be practised, and such modes or treatments may vary according to the character of the ore and the substance desired to be recovered. One possible mode of treatment is by electro-deposition, and to carry out that treatment I have provided supplemental tanks 17 and 50 18 arranged in descending series beside and below the tank 13. An overflow pipe 19 from the tank 13 discharges into tank 17, and a similar overflow pipe 20 from the top 55 of tank 17 discharges into tank 18. A pipe line 21 in which there is a pump 22 passes from the bottom of the tank 18 to a point whence it may discharge into the tank 13. The tanks are all provided with drain 60

70 pipes 23, 24, and 25, equipped with valves, whereby their contents may be withdrawn when required. In each of the tanks there are positive and negative electrodes 26 and 27, respectively, connected in circuit with any source of electrical energy capable of supplying current of proper tension. The purpose of this part of the apparatus is to recover metallic constituents of the ore from the liquor by electro-deposition, and the 75 character of the electrodes and of the electric currents supplied thereto is determined according to principles well known to those familiar with electro-deposition to the end that any metal which is a constituent of the ore may be extracted from the liquor in any selected tank by deposition on the electrodes in that tank.

The character of metals to be sought for by the electric action is determined by a preliminary assay of the ore, and it may also be determined with great accuracy by those skilled in the performance of the method, by a study of the colors of the volatilized ore in the arc.

90 One other possible mode of treatment of the solution than that of electro-deposition, by which also to secure the metals, consists in precipitating the liquor obtained from the condensing chamber by an alkaline reagent, drying the precipitate formed thereby, heating the precipitate in a crucible with a flux composed of carbonate of soda and borax and sometimes adding common sand. When the mass consisting of the mixture of the precipitate and of carbonate of soda and borax is heated until it becomes of a pasty consistency, the sand (when used) is added and the heating is continued until the mixture completely melts and becomes 95 liquid. Then the liquid is poured into a mold in which, before hardening, the metal settles to the bottom. The flux above mentioned is preferably made in the proportion of approximately one part of borax to two 100 parts of carbonate of soda, and common sand (when used) in quantities according to the ore. Some ores do not require sand.

105 By describing my method and apparatus thus particularly I have not intended to do more than illustrate the essential features of the invention. The process may be varied in many particulars in accordance with the ores treated, without departing from the spirit of the invention, and so also may the details of construction of the apparatus. Other products than merely metals as hereinbefore described may be obtained by proper modifications of the method, as for instance possibly metallic alloys, sulfur compounds, and acids or salts 110 of various sorts.

115 I have treated by the process hereinbefore described, many kinds of ores obtained from many widely separated parts of the 120 125 130

United States, Canada, and Mexico, containing not only the precious metals, but also lead, iron, zinc, arsenic, cobalt, sulfur, magnesia, lime and other metals and substances. In every instance the pulverized or granulated ore was fed into the electric arc, the ore was volatilized thereby, and the products of such volatilization were entrapped in an acid solution containing either hydrochloric acid, or a mixture of hydrochloric and nitric acids, as the acid principle, in substantially the proportions above named.

I have found as a result of my experience 15 and experiments that every kind of ore treated was volatilized and that substantially all of the volatile products coming in contact with the solvent were absorbed and retained in the solvent. I have also found 20 that some at least of the ingredients of the ores thus absorbed were so retained in the liquor as to be incapable of removal by mechanical means such as filtration. I have also succeeded in extracting the metals 25 sought for from the liquors so produced, by the methods hereinbefore described, and this is true in respect to even such ores as contained metals in chemical combination with other substances; at least to the extent that 30 in case of the ores last referred to I was able to recover the metals by precipitation and heating with borax and carbonate of soda. I have also found that it is possible to obtain a larger proportion of the metals 35 of all ores by my process than by any other known process, and that valuable by-products as well as metals are obtainable from ores treated by my method.

In the foregoing description and in the 40 following claims the terms "products of volatilization," "volatile products," "volatile matter," and "products from the furnace" are intended to include generically all the substances of gaseous or vaporous nature 45 which are developed, formed, or liberated by the action of the intense heat within the furnace upon the ore which is fed into the furnace, and include all gases of the metals or other constituents of the ore, whether elemental or in the same compounds as exist 50 in the original ore, or in combination with oxygen by reaction occurring at the time of volatilization.

What I claim and desire to secure by Letters Patent is:—

1. The method of producing a liquor containing in a dissolved condition the volatile products of minerals, which consists in heating the minerals to the point at which the 60 mineral is volatilized, and bringing the volatile matter as produced into intimate mixture with a solvent.

2. The method of producing a liquor containing in a dissolved condition the volatile 65 products of mineral ore, which consists in

heating the ore to a degree sufficient to volatilize and dissociate the minerals of the ore, conducting the volatile matter so liberated or produced, into contact with a solvent and causing such solvent to entrap and retain such volatile matter. 70

3. A process for the purpose indicated, which consists in feeding the ore into the region of an electric arc, whereby mineral is converted into gas, and intimately mingling such gas with liquid. 75

4. The method of producing a liquor containing constituents of a mineral ore in solution, which consists in heating the ore until volatile matter is produced, conducting such volatile matter as produced into contact with a solvent consisting mainly of acidulated water, and agitating such solvent while in contact with such volatile matter. 80

5. A process of treating ores which consists in volatilizing the ore by heat, collecting the volatilized products as produced in acidulated water, and further treating the liquor to extract constituents of the ore. 85

6. The method of treating metallic ores 90 which consists in volatilizing the ore in an electric arc, and entrapping the metallic constituents of the volatile matter produced thereby in a solvent consisting of water acidulated with hydrochloric acid. 95

7. The method of treating metallic ores which consists in volatilizing the ore in an electric arc, and collecting the metallic constituents of the volatile matter produced thereby in a solvent consisting of water acidulated with a mixture of hydrochloric and nitric acids. 100

8. The method of extracting metals from ores which consists in volatilizing the ore, intimately mingling the volatilized products, as produced, with a liquid, and extracting the metal from the liquid. 105

9. A process of separating mineral from the ore in which it occurs which consists in heating the ore to such a degree that it is volatilized and dissociated, absorbing the gas thus produced in a liquid while the gas is nascent, and separating the mineral from the liquor. 110

10. A process for separating metal from the natural substance in which it is found which consists in heating the natural substance to such a degree that the whole or a portion thereof is converted into gas, as produced, conducting the gas into intimate contact with a spray of dilute acid, precipitating the metallic matter absorbed by such acid by the action of an alkaline reagent, and melting the precipitate with a suitable flux. 115

11. A process of obtaining a specific substance from a mineral ore, which consists in heating the ore to such a degree that it is converted in part or in whole into gas, conducting the gas as produced into intimate 120

1 contact with a spray of dilute acid, and mixing the gas and acid thoroughly together.

12. A process for separating a metallic substance from the natural substance in

5 which it is found combined which consists in heating the natural substance to such a degree that the whole or a portion thereof is converted into gas, conducting the gas into intimate contact with a spray of dilute acid, precipitating the metallic matter dissolved in the acid by an alkaline reagent, and melting the precipitate with a suitable flux composed of carbonate of soda and borax.

15. 13. A process for separating metal from the natural substance in which it is found combined, which consists in heating the substance to such a degree that the whole or a portion thereof is converted into gas, conducting the gas into intimate contact with a spray of dilute acid, precipitating the metallic matter absorbed in the acid by an alkaline reagent, softening the precipitate, mixed with a flux consisting of borax and carbonate of soda, by heating to a pasty consistency, adding common sand, further heating the mixture until it has become liquid, and allowing the melted liquid to settle and cool.

30. 14. A method of treating ores which consists in feeding the ore in a finely divided condition to a region of high temperature, making such temperature of an intensity sufficient to convert the ore into a gaseous condition, collecting the gas while at the intensely high temperature, mixing the collected gas intimately with a liquid by means of a spray of the latter, and conducting the same liquid repeatedly into intimate relation with newly generated and collected gas.

15. The method of treating ores which consists in feeding the ore in a finely divided condition to a region of heat of an intensity and area sufficient to convert the ore into a gaseous condition, collecting the gases so produced, and injecting a spray of dilute acid into the space containing the collected gases, whereby such gases are condensed and absorbed by the acid.

50. 16. The method of obtaining liquor containing mineral substances, which consists in heating the raw material in which such substance is found to a degree sufficient to volatilize such substance, bringing the products of volatilization so produced into intimate mingled relation with a liquid, and agitating the liquid and products of volatilization together to cause absorption of the products of volatilization by the liquid.

60. 17. The method of producing a liquor containing the ingredients of metal bearing ore, which consists in heating raw ore to the point of volatilization, bringing the products of volatilization produced thereby into contact with a liquid which consists mainly

of acidulated water, and agitating the liquid and products of volatilization to cause absorption of the products of volatilization by the liquid.

18. The method of producing a liquor 70 containing metals in solution which consists in heating metal bearing ore to the temperature at which metal constituents thereof are volatilized, and conducting the volatile matter as produced into intimate mingled 75 relation with a solvent consisting of acidulated water.

19. The method of producing a liquor containing metals in solution which consists in heating metal bearing ore to the temperature 80 at which the metal constituents thereof are volatilized, and intimately mixing the volatile matter so produced while in the nascent condition, with a dilute aqueous solution of aqua regia.

20. The method of producing a liquor 85 containing precious metals in solution, which consists in heating ore containing such precious metals to the temperature at which such metals are volatilized, and mixing the volatilized metals intimately with dilute aqua regia, whereby such metals are to a considerable extent dissolved.

21. The method of treating metaliferous 95 ores which consists in volatilizing and dissociating metallic constituents of the ore by intense heat, and bringing the nascent gaseous substances thereby produced into intimate contact with an aqueous solution of nascent aqua regia.

22. The method of treating metaliferous 100 ores which consists in volatilizing the metallic constituents of the ore by intense heat, and bringing the gaseous substances produced by such volatilization while in a nascent condition into intimate mixture with an aqueous acid solution, whereby such gaseous substances are wholly or partially dissolved.

23. The method of treating ores which 105 consists in first heating such ores to the temperature of volatilization and dissociation of the constituents of the ore, and at once bringing the gases produced by such heating into intimate contact with relatively cold liquid.

24. The method of treating ores which 110 consists in first heating such ores to the temperature of volatilization and dissociation of the constituents of the ore, and at once bringing the gases produced by such heating into intimate contact with relatively cold liquid and agitating the liquid and gas together in a confined space.

25. An ore treating apparatus, comprising 115 heating means adapted to raise the temperature of ore to the point at which volatile matter is liberated from such ore, a collection chamber arranged to receive the volatile matter liberated by said heating 120

130

means, an injecting device for spraying a solvent into said chamber, and means for agitating the liquid and volatile matter together.

5 26. An ore treating apparatus, comprising heating means adapted to raise the temperature of ore to the point at which volatile matter is liberated from such ore, a collection chamber arranged to receive the volatile matter liberated by said heating means, an injecting device for spraying a solvent

into said chamber, a pump located and arranged to exhaust the liquid and gaseous matter from said chamber and being constructed to agitate the liquid and volatile 15 matter together.

In testimony whereof I have affixed my signature, in presence of two witnesses.

HIRAM E. TAYLOR.

Witnesses:

ARTHUR H. BROWN,  
P. W. PEZZETTI.